

1

3,346,386

## POLYCONDENSATION PRODUCTS OF PHOSPHORIC ACID AMIDES WITH ALIPHATIC POLYETHERS AS DEVELOPER ADJUVANTS

Herbert Müller, Leverkusen, Herbert Grabböfer, Cologne-Flittard, Hans Ulrich, Leverkusen, and Rolf-Fred Posse, Cologne-Flittard, Germany, assignors to Agfa Aktiengesellschaft, Leverkusen, Germany, a corporation of Germany

No Drawing. Filed Dec. 10, 1963, Ser. No. 329,364  
Claims priority, application Germany, Dec. 17, 1962,

A 41,899

5 Claims. (Cl. 96—66.3)

The invention relates to a process for the production of photographic images, the development of the exposed photographic material being carried out in the presence of polycondensation products of phosphoric acid amide derivatives with aliphatic polyethers. Phototechnical films of the so called litho- or line-type are increasingly being used in the reprography, in particular photo production of screened photographic prints. Litho- or line films are such films which can be developed in developer compositions containing formaldehyde bisulfite compounds to very high  $\gamma$ -values and thus to sharp screened dots. The term  $\gamma$  is to be understood as the tangent of the angle between the straight-line portion of the characteristic curve (or H and D curve) of the leg E axis.

It is true that processing of such films with formaldehyde-containing developers leads to excellent results, but the operation must be performed with great care, since the period during the development which yields a sharp screen dot, i.e., steepest gradation, is too brief, approximately between half and 1½ minutes.

It is known to add phosphorylated alkylene oxide derivatives to photographic silver halide emulsions to improve the mechanical properties. Such compounds are however, not operative for producing a steep gradation.

It is an object of the present invention to provide novel compounds which are added to the photographic layers or to the aqueous developing composition and with which an extremely high  $\gamma$ -value can be obtained upon development. A further object is to provide compounds which simultaneously effect the development in such a manner that the period of time during which that high  $\gamma$ -value is obtained can be extended so that the development is more convenient and simpler. Other objects, some of which are referred to specifically hereinafter will be evident to those skilled in the art to which this invention pertains.

These objects have been achieved by providing condensation products of aliphatic polyethers with terminal hydroxy groups and phosphoric acid amide derivatives of the formula



in which  $R_1$  represents an alkyl group preferably with up to 5 carbon atoms or an aryl, preferably phenyl or alkyl phenyl, or aralkyl, such as benzyl group;  $R_2$  can have the same meaning as  $R_1$  or can represent a hydrogen atom and  $X$  represents halogen atoms such as bromine or preferably chlorine, or alkoxy groups, preferably short-chain groups having up to 5 carbon atoms such as methoxy and ethoxy;  $R_1$  and  $R_2$  can be together the methylene groups to form a heterocyclic ring, in particular a piperidine or pyrrolidine ring.

Especially suitable polyethers are polyethyleneglycols which contain at least 3, preferably 4-10  $-\text{CH}_2\text{CH}_2\text{O}-$  units.

2

To produce the condensation products, 1 to 2 mols of polyether are advantageously reacted with 1 mol of the amido phosphoric acid compound. The following amido phosphoric acid compounds exhibit particular utility:

- 5  $\text{CH}_3\text{NHPOCl}_2$
- $\text{C}_2\text{H}_5\text{NHPOCl}_2$
- $\text{C}_3\text{H}_7\text{NHPOCl}_2$
- $\text{C}_5\text{H}_{11}\text{NHPOCl}_2$
- $\text{C}_6\text{H}_5\text{CH}_2\text{NHPOCl}_2$
- $\text{C}_6\text{H}_5\text{NHPOCl}_2$
- 10  $4\text{-ClC}_6\text{H}_4\text{NHPOCl}_2$
- $2,4\text{-Cl}_2\text{C}_6\text{H}_3\text{NHPOCl}_2$
- $2\text{-CH}_3\text{C}_6\text{H}_4\text{NHPOCl}_2$
- $2,3,5\text{-(CH}_3)_3\text{C}_6\text{H}_2\text{NHPOCl}_2$
- 15  $(\text{CH}_3)_2\text{NPOCl}_2$
- $(\text{C}_2\text{H}_5)_2\text{NPOCl}_2$
- $(\text{C}_2\text{H}_5)_2\text{NPOBr}_2$
- $(\text{iso-C}_4\text{H}_9)_2\text{NPOCl}_2$
- $(\text{C}_6\text{H}_5)\text{CH}_3\text{NPOCl}_2$
- 20  $(\text{C}_6\text{H}_5)\text{C}_2\text{H}_5\text{NPOCl}_2$
- $(\text{C}_6\text{H}_5)_2\text{NPOCl}_2$
- $\text{C}_5\text{H}_{10}\text{NPOCl}_2$
- $\text{CH}_3\text{NHPO}(\text{OC}_2\text{H}_5)_2$
- $\text{C}_2\text{H}_5\text{NHPO}(\text{OC}_2\text{H}_5)_2$
- 25  $\text{C}_3\text{H}_7\text{NHPO}(\text{OC}_2\text{H}_5)_2$
- $\text{iso-C}_4\text{H}_9\text{NHPO}(\text{OC}_2\text{H}_5)_2$
- $\text{C}_6\text{H}_5\text{NHPO}(\text{OCH}_3)_2$
- $\text{C}_6\text{H}_5\text{NHPO}(\text{OC}_2\text{H}_5)_2$
- $\text{C}_6\text{H}_5\text{NHPO}(\text{OC}_3\text{H}_7\text{-iso})_2$
- 30  $2,4\text{-Cl}_2\text{C}_6\text{H}_3\text{NHPO}(\text{OC}_2\text{H}_5)_2$
- $2\text{-CH}_3\text{C}_6\text{H}_4\text{NHPO}(\text{OC}_2\text{H}_5)_2$
- $(\text{CH}_3)_2\text{NPO}(\text{OCH}_3)_2$
- $(\text{C}_2\text{H}_5)_2\text{NPO}(\text{OCH}_3)_2$
- 35  $(\text{C}_3\text{H}_7)_2\text{NPO}(\text{OC}_2\text{H}_5)_2$
- $(\text{C}_4\text{H}_9)_2\text{NPO}(\text{OC}_4\text{H}_9)_2$
- $(\text{C}_6\text{H}_5)_2\text{NPO}(\text{OC}_2\text{H}_5)_2$

The aforesaid compounds are described, for example, in the article by A. Michaelis, Ann. volume 326, 129 (1903).

The products which are obtained by reaction of the above components and which are generally water-soluble, probably have the following structure:



in which  $R_1$  and  $R_2$  have the meanings indicated above, the integers  $n$ ,  $m$  and  $Z$  have the following meaning:

$m=0$  or at least 3, preferably 4-10;

$n=$  at least 3, preferably 4-10;

$Z=$  at least 1, preferably 1-1000.

The action of these compounds in connection with litho development was all the more unexpected because short-chain polyethylene glycols such as octaethylene glycol and even the analogous phosphoric and phosphorous acid polyethyleneglycol ester, as described in Belgian Patent 609,497, do not produce any sharp gradations. By the term litho development or litho developer we intend a development process which yields images with very steep gradation of at least 3 by the use of a developer which contains a formaldehyde-bisulfite compound.

Suitable for the process according to the invention are all silver halide emulsions which show a sufficiently high gradation effect with developers which contain formaldehyde.

The silver salts in such emulsions generally comprise at least 50 mol percent of silver chloride. For the process according to the invention, it is preferred to use emulsions, the silver halide of which contains at least 65 mol

percent of silver chloride and 35 mol percent or less silver bromide. The silver halide may further contain a small amount of up to 5 mol percent silver iodide.

The photographic silver halide emulsions produced can be sensitized with, for example, noble metal compounds or sulphur compounds.

About 0.1 to 10 grams of the phosphoric acid ester according to the invention can be added to the silver halide emulsions per kilogram of emulsion, the maximum quantity depending upon the ratio of chloride to bromide in the emulsion. It is advantageous to use from 10 to 100 mg. per mol of silver halide. The compounds are added to the developer solutions or to the emulsions, advantageously in quantities of 30 to 300 mg./liter of the emulsion-casting solution. The final dried silver halide emulsion layer with such addition accordingly contains between 0.5 and 10 mg. of the compound per square meter.

By the addition of the phosphoric acid amide esters of the present invention to the emulsion or to the developer, the  $\gamma$ -value in the development is shifted from about 6 to 8 to  $>15$ . Moreover, the period of development time during which the steepest gradation or screen dot sharpness is produced is raised from about 1 minute to 3 to 4 minutes. An additional advantage is that a developer containing formaldehyde is much less dependent upon temperature when it has such an additive. Whereas a developer without this additive reacts with a considerable development acceleration and thus a pronounced shortening of the development time when the temperature is raised by 1 to  $2^\circ$ , good results are obtained with a developer temperature between 15 and  $40^\circ$  when phosphoric acid amide esters are added. Because of the longer processing period, the advantages described above lead to much more reliable working. The compounds according to the invention can be added to the developer composition in an amount of 0.01 to 10 grams per liter of the aqueous composition.

The phosphoric acid amide esters according to the invention are prepared by conventional esterification methods; the degree of condensation of the ester can be influenced as required by variations in the reaction time and in the reaction temperature. The higher the temperature, the higher is the degree of condensation of the phosphoric acid amide esters, in particular the integer "Z" of the polyether ester formula can be influenced by varying the temperature. Thus, compounds were obtained in which Z had a value of about 100, 300, 800 or 1000. The degree of condensation can further be influenced, in particular the integer Z referred to hereinbefore, by varying the proportion of the starting compounds for the condensation. Compounds with a very high value of Z having repeating phosphoric acid amide units in a wholly ether chain are obtained if the phosphoric acid amide reactant and the aliphatic polyether are reacted in a molar proportion of 1:1. Compounds containing only 1 phosphoric acid amide grouping are obtained if the phosphoric acid amide reactant and the polyether are reacted in a molar proportion of 1:2.

In the following examples concerned with production, a number of condensation products are separately described:

#### COMPOUND I

19 g. of N,N-diethylphosphoric acid amide-dichloride are added in portions at temperatures between 0 and  $5^\circ$  C., while stirring to a mixture of 31.2 g. of pyridine and 28.2 g. of hexaethylene glycol. The mixture is left standing for 5 hours at room temperature and is then poured onto ice, acidified with 2 N-sulphuric acid and extracted with methylene chloride. After drying with potash, the methylene chloride is completely evaporated. There are obtained 39 g. of a syrupy amber-coloured substance.

#### COMPOUND II

41.2 g. of nonaethylene glycol, 31.2 g. of pyridine and 19 g. of N,N-diethyl phosphoric acid amide-dichloride are reacted and worked up in the manner described above.

There are obtained 45 g. of a semi-solid, brown-coloured substance, which is diluted with water to a 10% solution and purified with activated carbon.

#### COMPOUND III

The preparation is similar to that of compound (I), by reaction of 28.2 g. of hexaethylene glycol, 31.2 g. of pyridine and 22.4 g. of N-methyl-N-phenyl phosphoric acid amide dichloride. There are obtained 39 g. of a brown-coloured, semi-solid substance, which is purified with activated carbon.

#### COMPOUND IV

41.4 g. of nonaethylene glycol, 31.2 g. of pyridine and 22.4 g. of N-methyl-N-phenyl phosphoric acid amide-dichloride are reacted in a manner analogous to Compound I. There are formed 50 g. of a brown-coloured semi-solid substance, which is diluted with water and decoloured with activated carbon.

#### COMPOUND V

1 mol of propylamidophosphoric acid diethyl ester is heated with approximately a 10% molar excess of octaethylene glycol in the presence of reesterification catalysts, such as sodium or sodium alcoholate, for several hours at 100 to  $120^\circ$  C. The ethyl alcohol that is liberated is constantly distilled off in vacuo and the residue can be used for the purpose of the present invention.

#### Example 1

A gelatino-silver halide emulsion with 15 mol percent of AgBr and 85% of AgCl is washed, ripened to the maximum sensitivity and, after adding 4-hydroxy-6-methyl-1,3,3a,7-tetrazaindol or other stabilisers and a wetting agent, cast onto a suitable film support.

Other film strips are prepared with the use of the same emulsions, 80 mg. of octaethylene glycol or 80 mg. of the Compounds I-IV according to the invention being added to separate portions of the casting mixture. All specimens are exposed behind a grey stepped wedge and developed for 5 minutes in a developer with the following composition at  $18^\circ$ .

|                                | Grams |
|--------------------------------|-------|
| Anhydrous sodium sulphite      | 30    |
| Boric acid                     | 7.5   |
| Hydroquinone                   | 22.5  |
| Potassium metabisulphite       | 2.5   |
| Paraformaldehyde               | 7.5   |
| Potassium bromide              | 1.5   |
| Made up with water to 1 litre. |       |

In the sensitometric evaluation of the film strips, the following results are obtained:

|                     | Emulsion additive | Gradation | Fogging |
|---------------------|-------------------|-----------|---------|
| Octaethylene glycol | 6                 | 0.04      |         |
| Compound I          | $>15$             | 0.04      |         |
| Compound II         | $>15$             | 0.04      |         |
| Compound III        | $>15$             | 0.04      |         |
| Compound IV         | $>15$             | 0.04      |         |

#### Example 2

Film strips of the emulsion described in Example 1 are exposed behind a grey stepped wedge and are developed 70 in the developer referred to above for periods from 1 to 6 minutes (Experiment A). The same film specimens, after addition of 100 mg. of the Compound I (Experiment B) and 100 mg. of the phosphorous acid glycol ester according to Example 1 of Belgian Patent 609,497 (Experiment C), 75 are developed in the same developer.

|   | Result                                       |                                                   |                                                     |                                                        |                                                        |                                                        | 6 |
|---|----------------------------------------------|---------------------------------------------------|-----------------------------------------------------|--------------------------------------------------------|--------------------------------------------------------|--------------------------------------------------------|---|
|   | 1.5                                          | 2                                                 | 2.5                                                 | 3                                                      | 4                                                      | 5                                                      |   |
| A | 1.5<br>(Time, Minutes)<br>( $\gamma$ -value) | 2<br>>10<br>(Time, Minutes)<br>( $\gamma$ -value) | 2.5<br>>10<br>(Time, Minutes)<br>( $\gamma$ -value) | 3<br>6<br>>10<br>(Time, Minutes)<br>( $\gamma$ -value) | 4<br>6<br>>10<br>(Time, Minutes)<br>( $\gamma$ -value) | 5<br>6<br>>10<br>(Time, Minutes)<br>( $\gamma$ -value) | 6 |
| B | 1.5<br>(Time, Minutes)<br>( $\gamma$ -value) | 2<br>>10<br>(Time, Minutes)<br>( $\gamma$ -value) | 2.5<br>>10<br>(Time, Minutes)<br>( $\gamma$ -value) | 3<br>8<br>>10<br>(Time, Minutes)<br>( $\gamma$ -value) | 4<br>5<br>>10<br>(Time, Minutes)<br>( $\gamma$ -value) | 5<br>6<br>>10<br>(Time, Minutes)<br>( $\gamma$ -value) | 6 |
| C | 1.5<br>(Time, Minutes)<br>( $\gamma$ -value) | 2<br>>10<br>(Time, Minutes)<br>( $\gamma$ -value) | 2.5<br>>10<br>(Time, Minutes)<br>( $\gamma$ -value) | 3<br>8<br>>10<br>(Time, Minutes)<br>( $\gamma$ -value) | 4<br>6<br>>10<br>(Time, Minutes)<br>( $\gamma$ -value) | 5<br>6<br>>10<br>(Time, Minutes)<br>( $\gamma$ -value) | 6 |

## Example 3

An emulsion as in Example 1 is given the usual additives (wetting agents, stabilisers and hardeners) and is divided into three portions and cast as follows onto a film support:

A: Without additive

B: +80 mg. of the Compound II per mol of silver halide  
C: +80 mg. of the analogous phosphoric acid glycol ester according to Example 3 of Belgian Patent No. 609,497.

Several samples are cut from these webs and exposed in a sensitometer behind a grey stepped wedge and developed as follows in the aforementioned developer at 18° C.:

|   | Time, Minutes                       | 1.5       | 2        | 2.5        | 3      | 4      | 5      | 6 |
|---|-------------------------------------|-----------|----------|------------|--------|--------|--------|---|
| A | Time, Minutes<br>( $\gamma$ -value) | 1.5<br>10 | 2<br>>10 | 2.5<br>>10 | 3<br>6 | 4<br>6 | 5<br>6 | 6 |
| B | Time, Minutes<br>( $\gamma$ -value) | 1.5<br>8  | 2<br>10  | 2.5<br>>10 | 3<br>8 | 4<br>5 | 5<br>6 | 6 |
| C | Time, Minutes<br>( $\gamma$ -value) | 1.5<br>10 | 2<br>>10 | 2.5<br>>10 | 3<br>6 | 4<br>6 | 5<br>6 | 6 |

We claim:

1. In a process for developing an exposed photographic material containing at least 1 silver halide emulsion layer, the silver halide of which contains at least 50 mol percent of silver chloride, in a photographic aqueous developer composition containing formaldehyde, the improvement which consists in developing the exposed photographic material in contact with a reaction product of 1 to 2 mols of aliphatic polyether having terminal hydroxy groups, and 1 mol of a phosphoric acid amide derivative of the formula



in which  $R_1$  is a radical of the group consisting of alkyl, phenyl, alkyl phenyl and phenyl alkyl;  $R_2$  is a substituent of the group consisting of hydrogen, alkyl, phenyl, alkyl phenyl and phenyl alkyl or  $R_1$  and  $R_2$  together are the methylene groups required to complete a heterocyclic radical of the group consisting of pyrrolidino and piperidino and  $X$  represents a substituent of the group consisting of chlorine, bromine and lower alkoxy.

2. A process as defined in claim 1, in which the reaction products has the following formula:



wherein  $R_1$  and  $R_2$  have the meaning defined in claim 1,  $m$  can be 0 and an integer from 3 to 10;  $n$  is an integer from 3 to 10 and  $Z$  is an integer from 1 to 1000.

3. A process as defined in claim 1, wherein the reaction product has the following formula



wherein  $R_1$  and  $R_2$  have the meaning defined in claim 1,  $m$  is an integer from 4 to 10;  $n$  is an integer from 4 to 10 and  $Z$  is an integer from 1 to 1000.

4. A light-sensitive photographic material having at least one light-sensitive silver halide emulsion layer and containing between 0.1 and 10 grams per kilogram of the compound of the following formula



wherein  $R_1$  and  $R_2$  have the meaning defined in claim 1,  $m$  can be 0 and an integer from 3 to 10;  $n$  is an integer from 3 to 10 and  $Z$  is an integer from 1 to 1000.

5. An aqueous composition containing a silver halide photographic developer and from 0.01 to 10 grams per liter of a compound of the following formula:



wherein  $R_1$  and  $R_2$  have the meaning defined in claim 1,  $m$  can be 0 and an integer from 3 to 10;  $n$  is an integer from 3 to 10 and  $Z$  is an integer from 1 to 1000.

## References Cited

## UNITED STATES PATENTS

- 3,156,718 11/1964 Lorenz et al. ----- 260-461  
3,157,685 11/1964 Szabo et al. ----- 260-461  
3,158,483 11/1964 Lowe et al. ----- 96-66  
3,162,534 12/1964 Powers et al. ----- 96-66

NORMAN G. TORCHIN, Primary Examiner.

C. E. DAVIS, Assistant Examiner.